

# UNITED STATES PATENT OFFICE.

EMIL F. DIETERICH, OF PHILADELPHIA, PENNSYLVANIA.

## IMPROVEMENT IN WATER-REPELLENT DUBBING FOR LEATHER.

Specification forming part of Letters Patent No. 150,303, dated April 28, 1874; application filed April 15, 1874.

*To all whom it may concern:*

Be it known that I, EMIL F. DIETERICH, of Philadelphia, Pennsylvania, have invented a Water-Repellent Dubbing, of which the following is a specification:

Leather, after being tanned and dried and not otherwise finished, retains a rigidity which increases with time, and to counteract which it is necessary to grease or dub the leather.

The dubbings commonly employed for this purpose consist of oils more or less mixed with tallow, or sometimes with tallow and rosin, and often with tallow, wax, rosin, and other ingredients, the whole suspended in some drying or volatile oil. Even the well-known "French degras" is seldom used without a large admixture of tallow.

The benefits of such dubbings last only until the decomposition of their component parts has taken place. This decomposition rapidly results from the changes from moisture to dryness, or vice versa, undergone by the leather. In the case of boots and shoes it is occasioned by the perspiration of the feet, or in case of harness by perspiration from the body of the animal, or in either case it results from the ammonia in rain and snow water, and in all cases from many other influences, not only during use, but also during storage. When the dubbing has become thus decomposed the leather hardens and rots.

The composition which I prepare for dubbing and stuffing leather differs from those above mentioned by being entirely free from rosin, wax, tallow, and any of the drying or volatile oils. It is composed of insoluble water-repellent and pliant ingredients only, which settle around the fibers, protect them and render the leather water-repellent and permanently soft and pliable.

This water-repellent dubbing I prepare by heating neat's-foot oil, or other fatty matter of similar nature, until all moisture is expelled from it and its gluten has been destroyed, and I then dissolve in it caoutchouc in a divided

state, from eight to sixteen ounces to the gallon of fatty matter.

When it is desired to accelerate the process of mixing the caoutchouc with the fatty matter, and also to preserve the light color of the mixture, I use caoutchouc which has been previously softened by volatile hydrocarbon, and after mixing this thoroughly with the heated fatty matter, I continue applying heat by means of a water-bath, until all the hydrocarbon is evaporated and a uniform mixture of the caoutchouc and fatty matter obtained.

For denser compounds, such as are required when the dubbing is intended for stuffing process employed in finishing leather, I add to the mixture obtained by either of the above-described processes paraffine or crude stearine (such as is pressed from crude lard,) or a mixture of both, as much as twenty per cent. In this case the caoutchouc may be dissolved in the paraffine or stearine by the aid of heat, and then mixed with the heated fatty matter. To the oily compound thus formed I now add a portion of the oleate, stearate, margarate, or palmetate of alumina, (which are compounds insoluble in water,) in the proportion of from two to eight ounces of any of the alumina compounds to sixteen ounces of the oily compound, and maintain heat until all moisture is expelled and a uniform combination obtained.

Instead of the fatty acids last mentioned, any other fatty acid may be substituted.

I claim—

As a new manufacture, water-repellent dubbing, composed of fatty matter, caoutchouc, and a compound of alumina insoluble in water, with or without paraffine or stearine, all in the proportions mentioned, substantially as set forth.

E. F. DIETERICH.

Witnesses:

THOS. A. BURTT,  
JNO. A. BELL.